

**3,255,107**  
**FINISH COMPOSITION FOR POLYOLEFIN FIBERS**

Ann S. Keller, Norristown, and Harry H. Hall, Springfield, Pa., assignors, by mesne assignments, to FMC Corporation, San Jose, Calif., a corporation of Delaware

No Drawing. Filed Apr. 19, 1962, Ser. No. 188,839

8 Claims. (Cl. 252—8.75)

This invention relates to finished polyolefin fibers. More particularly, it relates to polyolefin yarns or fibers having applied finishes which enable the yarns to be satisfactorily processed and utilized in the commercial production of textiles and in machine sewing operations.

Polyolefin yarns, for example, polypropylene and polyethylene yarns, tend to develop high electrostatic charges and excessive tensions when running over guides, godets, and other objects during processing and subsequent handling. The utilization of unfinished polyolefin yarn in textile production and sewing equipment is unsatisfactory.

Static and tension problems have been encountered in the use of other natural and synthetic polymer yarns, and finishes which are satisfactory from both the standpoints of application and use have been developed for them. However, the polyolefins have different physical characteristics than most other filament forming polymers and conventional finishes and methods for application thereof are not suitable or effective in providing the necessary fiber to fiber lubrication, proper fiber to metal frictional behavior, and adequate static suppression.

A primary object of this invention is to provide a finished polyolefin yarn which is suitable for high speed processing, textile and sewing operations.

It is another object of this invention to provide a method of finishing polyolefin fibers which is effective in providing fiber lubrication and static suppression.

These and other objects are accomplished in accordance with this invention with a finish composition for polyolefin fibers consisting essentially of from about 1 to 5% by weight of a di C<sub>1</sub>—C<sub>6</sub> alkyl cyclohexyl amine salt of a C<sub>10</sub>—C<sub>18</sub> fatty acid sulfate, and a completely esterified C<sub>10</sub>—C<sub>18</sub> fatty acid ester of pentaerythritol. The C<sub>1</sub>—C<sub>6</sub> alkyl groups of the cyclohexyl amine salt include for example, methyl, ethyl, propyl, butyl, amyl, hexyl, and isomers of these groups. The C<sub>10</sub>—C<sub>18</sub> fatty acids for both the fatty acid sulfate radical of the amine salt and for the fatty acid ester portion of the pentaerythritol ester include for example, capric acid, lauric acid, myristic acid, palmitic acid, stearic acid, oleic acid, linoleic acid, etc. The completely esterified pentaerythritol laurate is the preferred pentaerythritol ester of this invention on the basis of availability and performance as a polyofin fiber lubricant.

The invention also includes polyolefin fibers, for example, polyethylene, polypropylene and polyisobutylene fibers having incorporated thereon the above described finish composition, and a method for the application of the finish to the fiber. The method of preparing finished polyolefin fibers comprises applying to said fibers the above described finish composition in the absence of water and a hydrocarbon oil. The fibers of this invention may be in the form of continuous monofilaments, multifilaments, staple, etc. The finished yarn or fiber may be scoured in the usual manner after processing or the yarn may be used in further textile operations with the finish remaining on the fiber, as desired.

Many lubricant antistat combinations were investigated to develop a satisfactory finish composition for polyolefin fiber. Before combinations of lubricants and antistats were tried, however, a screening test was conducted to determine whether the lubricant or antistat material would degrade the polyolefin. Screening involved placing approximately 0.2 ml. of the liquid lubricant or antistat onto

a sheet of polypropylene film which had been secured to a glass plate. A piece of graph paper was placed between the film and the glass and served two purposes; it would indicate penetration of the film by the liquid; and also give an indication of the spreading action of the lubricant or antistat. The material passed the screening test if 24 hours of film contact produced no change in film appearance such as waviness or puckering. If puckering did occur it was assumed that it was caused by penetration of the lubricant or antistat into the film and this type of behavior would also occur with a polypropylene fiber. Puckering was considered to be caused by plasticization or a similar phenomenon and test materials causing it were rejected.

The above screening test indicated that paraffinic oils and low molecular weight esters had a noticeable undesirable effect on the test film. Applications of these materials to polyolefin yarn at spinning and the consequential softening or plasticization of this yarn corroborated the screening test results.

To demonstrate the specificity of this invention there is set forth in the following table a list of finishes, the components of which have passed screening tests but which have been found unsatisfactory either in their application or in their ability to improve characteristics of the yarn.

TABLE I

| No. | Finish Composition                                     | Percent By Weight |
|-----|--------------------------------------------------------|-------------------|
| 30  | Diethyl cyclohexylamine salt of lauryl sulfate.        | 3-5               |
| 1.  | Coconut oil.                                           | 95-97             |
| 2.  | Diethyl cyclohexylamine salt of lauryl sulfate.        | 3-10              |
|     | Sorbitan monooleate.                                   | 1.5-5             |
| 3.  | Butyl stearate.                                        | 85-95.5           |
|     | Diethanolamine salt of diaryl phosphate.               | 3                 |
| 35  | Sorbitan monooleate.                                   | 4                 |
|     | Butyl Stearate.                                        | 93                |
| 4.  | 1-hydroxyethyl-2-oleyl ethyl glyoxolinium ethosulfate. | 3                 |
|     | Sorbitan monooleate.                                   | 3                 |
| 5.  | Butyl stearate.                                        | 94                |
|     | Sorbitan monooleate.                                   | 5                 |
| 40  | Butyl stearate.                                        | 95                |
| 6.  | 1-hydroxyethyl-2-oleyl ethyl glyoxolinium ethosulfate. | 3                 |
|     | Sorbitan monooleate.                                   | 4                 |
|     | Coconut oil.                                           | 93                |
| 7.  | 1-hydroxyethyl-2-oleyl ethyl glyoxolinium ethosulfate. | 5                 |
|     | Sorbitan trioleate.                                    | 20                |
| 45  | Esterified pentaerythritol.                            | 75                |
| 8.  | Diethyl cyclohexylamine salt of lauryl sulfate.        | 10                |
|     | Water.                                                 | 90                |
| 9.  | Diethyl cyclohexylamine salt of lauryl sulfate.        | 10                |
|     | Diethyl glycol.                                        | 90                |
| 10. | Diethyl cyclohexylamine salt of lauryl sulfate.        | 5                 |
|     | Polyethylene glycol (M.W. 400) monooleate.             | 95                |
| 11. | Diethyl cyclohexylamine salt of lauryl sulfate.        | 5                 |
|     | Dialiphatic ether of polyethylene glycol.              | 95                |
| 12. | Esterified pentaerythritol.                            | 60                |
|     | Nonionic emulsifying agents.                           | 40                |
| 13. | Finish No. 12.                                         | 10                |
|     | Water.                                                 | 90                |
| 14. | Finish No. 12.                                         | 95                |
|     | Sorbitan monooleate.                                   | 3                 |
| 55  | N-cetyl N-ethyl morpholinium ethosulfate.              | 2                 |
| 15. | Finish No. 14.                                         | 20                |
|     | Water.                                                 | 80                |
| 16. | N-cetyl N-ethyl morpholinium ethosulfate.              | 5                 |
|     | Technical grade octanol.                               | 95                |
| 17. | N-cetyl N-ethyl morpholinium ethosulfate.              | 10                |
|     | Water.                                                 | 90                |
| 18. | N-cetyl N-ethyl morpholinium ethosulfate.              | 10                |
|     | Diethylene glycol.                                     | 90                |
| 60  | N-cetyl N-ethyl morpholinium ethosulfate.              | 2                 |
| 19. | Finish No. 12.                                         | 98                |
| 20. | Polyoxyethylene modified tallow acid primary amine.    | 5                 |
|     | Polyethylene glycol (M.W. 200) monolaurate.            | 95                |
| 21. | Polyethylene glycol (M.W. 200) monopalarnonate.        | 100               |
| 22. | Polyethylene glycol (M.W. 1000) monostearate.          | 2                 |
|     | Polyethylene glycol (M.W. 200) monopalarnonate.        | 98                |
| 23. | Diethanolamine salt of diaryl phosphate.               | 5                 |
|     | Finish No. 22.                                         | 95                |
| 24. | Diethanolamine salt of diaryl phosphate.               | 10                |
|     | Polyethylene glycol (M.W. 200) monopalarnonate.        | 90                |
| 25. | Polyethylene glycol (M.W. 400) monopalmitate.          | 2                 |
|     | Water.                                                 | 98                |
| 70  | Diethanolamine salt of diaryl phosphate.               | 10                |
| 26. | Polyethylene glycol (M.W. 200) monolaurate.            | 90                |

In addition to the above yarn finish compositions, many other unsatisfactory combinations were tested which were identifiable only under chemical tradenames and/or broad chemical terms.

Polyolefin fibers and in particular polypropylene fibers are much more difficult to finish than other synthetic or natural polymer fibers. They are non-polar materials and as such have no affinity for the usual yarn finishes. They are hydrophobic and in general, water base finish compositions cannot be used to obtain a satisfactory finish. The polyolefin fibers are degraded by treatment with hydrocarbon oil base compositions and become undesirably soft. For these reasons, the finish composition is extremely critical in order to obtain satisfactory yarn characteristics.

The following example is set forth to demonstrate finish application and composition in accordance with the invention.

*Example*

A finish comprising 2% by weight of diethyl cyclohexyl amine salt of lauryl sulfate and 98% of the completely esterified lauric acid ester of pentaerythritol was prepared. This finish was applied to polypropylene approximately 800 denier, 34 filament yarn just prior to the primary take-up by means of a kiss roll 6 inches in diameter and 1½ inches wide. The finish permitted the yarn to be collected onto a standard take-up tube with ease. Moreover, it was a definite aid in processing the yarn through a draw-twisting operation.

Various changes and modifications may be made in practicing the invention without departing from the spirit and scope thereof and, therefore, the invention is not to be limited except as defined in the appended claims.

We claim:

1. A finish composition for polyolefin fibers consisting of from about 1 to 5% by weight of a di-C<sub>1</sub>-C<sub>6</sub> alkyl cyclohexyl amine salt of a C<sub>10</sub>-C<sub>18</sub> fatty acid sulfate, and a completely esterified C<sub>10</sub>-C<sub>18</sub> fatty acid ester of pentaerythritol.

2. The finish composition of claim 1 wherein the cyclohexyl amine salt is diethyl cyclohexyl amine salt of lauryl sulfate.

3. The finish composition of claim 1 wherein the pentaerythritol ester is the lauric acid ester of pentaerythritol.

4. A polyolefin fiber having incorporated thereon a finish consisting of from about 1 to 5% by weight of a di-C<sub>1</sub>-C<sub>6</sub> alkyl cyclohexyl amine salt of a C<sub>10</sub>-C<sub>18</sub> fatty acid sulfate, and a completely esterified C<sub>10</sub>-C<sub>18</sub> fatty acid ester of pentaerythritol.

10 5. The polyolefin fiber of claim 4 wherein the cyclohexylamine salt is diethyl cyclohexyl amine salt of lauryl sulfate.

15 6. The polyolefin fiber of claim 4 wherein the pentaerythritol ester is the lauric acid ester of pentaerythritol.

7. The method of preparing finished fibers which comprises treating polyolefin fibers with a finish in the absence of water and hydrocarbon oil, said finish consisting of from about 1 to 5% by weight of a di-C<sub>1</sub>-C<sub>6</sub> alkyl cyclohexyl amine salt of a C<sub>10</sub>-C<sub>18</sub> fatty acid sulfate, and a completely esterified C<sub>10</sub>-C<sub>18</sub> fatty acid ester of pentaerythritol.

20 8. The method of claim 7 wherein polypropylene fibers are treated with a finish consisting of from about 1 to 5% by weight of diethyl cyclohexyl amine salt of lauryl sulfate and the lauric acid ester of pentaerythritol.

**References Cited by the Examiner**

**UNITED STATES PATENTS**

|              |         |                  |       |          |
|--------------|---------|------------------|-------|----------|
| 30 2,139,276 | 12/1938 | Lehrer et al.    | ----- | 252—8.75 |
| 2,191,033    | 2/1940  | Faw              | ----- | 252—8.75 |
| 2,597,947    | 3/1952  | Oxlev et al.     | ----- | 252—8.75 |
| 2,614,984    | 10/1952 | Thomas et al.    | ----- | 252—8.75 |
| 35 2,668,785 | 2/1954  | Jefferson et al. | ----- | 252—8.75 |
| 3,009,830    | 11/1961 | Levine           | ----- | 252—8.9  |

JULIUS GREENWALD, *Primary Examiner*.

J. T. FEDIGAN, *Assistant Examiner*.